

June 20, 1939.

C. DE ROHDEN

2,162,942

C. DE ROHDEN  
PROCESS FOR THE PREPARATION OF MAGNESIUM BY  
THE ELECTROLYSIS OF ITS FUSED CHLORIDE  
Filed July 14, 1936



Charles de Rohden,  
INVENTOR  
by Foster & Codier  
ATTORNEYS

## UNITED STATES PATENT OFFICE

2,162,942

## PROCESS FOR THE PREPARATION OF MAGNESIUM BY THE ELECTROLYSIS OF ITS FUSED CHLORIDE

Charles de Rohden, Neuilly-sur-Seine, France

Application July 14, 1936, Serial No. 90,579  
In Germany July 20, 1935

2 Claims. (Cl. 204—19)

When a mixture of fused salts containing magnesium chloride together with the chlorides of the alkali and alkaline earth metals is electrolysed, the electrolyte becomes poorer in magnesium chloride and richer in the other constituents. The electrolyte also becomes richer in impurities and particularly in MgO. This latter impurity is not only introduced together with the dehydrated magnesium chloride serving for the electrolysis, but is also formed during the electrolysis if small quantities of water are present in or come into the electrolyte.

The preparation of pure anhydrous magnesium chloride is in general too complicated and costly for this substance to be employed for the electrolytic preparation of magnesium, and heretofore it has been the general practice to proceed by one of two well-known methods.

In the first of these methods a mixture of chlorides is electrolysed until the magnesium chloride content of the bath has sunk so low as to make further electrolysis inadvisable. In the second method the impoverished electrolyte is withdrawn from time to time without interrupting the electrolysis, whereupon the electrolytic cell is filled with a previous charge of the electrolyte so withdrawn which has subsequently been enriched with magnesium chloride. If said first method is employed, it is necessary to start with an electrolyte containing a relatively high percentage of magnesium chloride, as otherwise the labour involved in charging and discharging the cell becomes altogether disproportionate to the yield of metal. It is therefore impossible by this method to electrolyse with industrial success a mixture of salts containing less than 20% of magnesium chloride, which is the optimum value when current and energy efficiency are considered. The same considerations apply in a lesser degree to the said second method, which presents the added disadvantage that the solid impurities, and particularly the MgO, tend constantly to accumulate. Furthermore, both the aforesaid methods present the grave drawback that the level of the electrolyte in the cell varies with the progress of the electrolysis, thus causing variations in the anodic current density and accelerating the destruction of the anodes.

The object of the present invention consists in a process for the electrolytic preparation of magnesium from a bath containing fused magnesium chloride, which process eliminates the disadvantages enumerated above and permits of the electrolysis being carried out under the optimum conditions.

The invention furthermore permits of reducing the labour to a minimum, since it works continuously.

The invention consists essentially in making a series of electrode systems act in succession upon an electrolyte in motion, fresh electrolyte being continuously added so as to maintain an approximately constant level in each one of the electrolytic cells. The impoverished electrolyte leaving the last electrode system is preferably enriched with magnesium chloride and returned to the first electrode system.

This method of working permits of approaching the optimum conditions for the electrolysis. The continuous and carefully regulated entry and corresponding exit of the electrolyte maintain the level of the latter practically constant, thus prolonging the life of the anodes. Each system of electrodes continuously electrolyses a bath in which the magnesium chloride content at any point is kept practically constant, and the difference in concentration between each succeeding electrode system may, if so desired, be maintained slight, becoming less the greater the speed of circulation. This permits of obtaining and maintaining the optimum electrolytic conditions in each electrode system, and among others of maintaining the magnesium chloride content of the bath in each electrode system at less than 30%, and preferentially at less than 20%.

In order to put the invention into practice, it is possible to employ either a series of cells, or an unique cell in which several series of electrode systems act one after the other upon the electrolyte as it traverses the cell. In both cases the electrolytic cells are fed, either directly or indirectly, by means of a suitably heated container to which the impoverished electrolyte is returned, and where it is enriched in MgCl<sub>2</sub> before being returned to the cycle. This enriching of the impoverished electrolyte may be carried out in any known manner, but it is the preferred practice to add, either continuously or discontinuously and in the solid or the fused state, a product consisting principally of hydrated MgCl<sub>2</sub> and of a composition approaching the tetrahydrate, until the enriched electrolyte contains about 30% of anhydrous MgCl<sub>2</sub>.

This mode of realization however presents the disadvantage that the electrolysis must be interrupted when the solid impurities, and especially the MgO, have accumulated sufficiently to interfere with the efficient working of the cells. In order to avoid this undesirable interruption of

the electrolysis, another suitably heated container is introduced into the system between the container where the impoverished electrolyte is enriched and the electrolytic cells in which the magnesium is produced. The enriched electrolyte is then allowed to decant in known manner and settle out its solid impurities in this intermediary container. A plant for the electrolytic production of magnesium thus equipped can work 10 efficiently for an indefinite period without being stopped.

The figure attached shows in diagrammatic vertical section the principal means of execution whereby the invention may be put into effect, 15 but it must be clearly understood that the means described are in no way to be construed as limiting the scope of the invention. *a* is a suitably heated container wherein the electrolyte is decanted from solid impurities in suspension. The 20 electrolyte is then fed discontinuously to the heated container *b* from which it is admitted, by means of a constant feed *c* to the first of a series of electrolytic cells *d* each having a cathode *e* and an anode *f*. The electrolyte overflows from 25 cell to cell through the orifices *h*, being finally admitted to the suitably heated container *g*, to which  $MgCl_2 \cdot 4H_2O$  is also fed at a constant rate so chosen as to ensure a bath having a composition approximating to 30%  $MgCl_2$ . The electrolyte 30 is then transferred discontinuously from *g* to the decantation cell *a* from whence it continues the previously described cycle.

It is moreover possible to put the invention into efficient practice even if the enriched electrolyte is not absolutely anhydrous. To this end the intermediary decantation container is suitably heated so as to eliminate the water present in the electrolyte to be fed to the electrolytic cells. Or again a slightly hydrous enriched electrolyte is submitted in known manner to a preliminary electrolysis under such working conditions of voltage and amperage that the water is decomposed without substantial decomposition of the magnesium chloride. When working the 45 process in this manner, it is advantageous to equip the container in which the solid impurities are decanted with means whereby the water is electrolysed.

The invention can moreover be put into practice with pure magnesium chloride, or any bath containing workable mixtures of magnesium chloride with the chlorides of more electropositive

metals. Nevertheless the advantages of the present invention are most marked when electrolysing a bath containing less than 30% magnesium chloride.

I claim:

1. A process of continuously producing magnesium by electrolysis of magnesium chloride in a fused electrolyte containing magnesium chloride and a chloride of a more electro-positive metal than magnesium, and in which the magnesium chloride is not in excess of 30% of the entire electrolyte, which comprises flowing said fused electrolyte in contact with a plurality of pairs of electrodes, while maintaining the level of the bath in contact with each particular pair of electrodes substantially constant, maintaining on each pair of electrodes a difference of potential sufficient to insure electrolysis of magnesium chloride with the production of magnesium, maintaining a continuous flow of said fused electrolyte in contact 15 with said pairs of electrodes until the content of magnesium chloride therein has been substantially reduced but not eliminated, adding a quantity of hydrated magnesium chloride corresponding substantially to the formula  $MgCl_2 \cdot 4H_2O$  to said 20 electrolyte, allowing sedimentation of magnesium oxide from said mixture and reintroducing the so-clarified and reinforced electrolyte to said 25 treatment.

2. A process of continuously producing magnesium by electrolysis of magnesium chloride in a fused electrolyte containing magnesium chloride and a chloride of a more electro-positive metal than magnesium, and in which the magnesium chloride is not in excess of 30% of the entire electrolyte, which comprises flowing said fused electrolyte in contact with a plurality of pairs of electrodes, while maintaining the level of the bath in contact with each particular pair of electrodes substantially constant, maintaining on each pair of electrodes a difference of potential sufficient to insure electrolysis of magnesium chloride with the production of magnesium, maintaining a continuous flow of said fused electrolyte in contact 35 with said pairs of electrodes until the content of magnesium chloride therein has been substantially reduced but not eliminated, adding a quantity of hydrated magnesium chloride to said electrolyte, allowing sedimentation of magnesium oxide from said mixture and reintroducing the so-clarified and reinforced electrolyte to said 40 treatment.

CHARLES DE ROHDEN.